

Oct. 3, 1972

K. J. BRONDYKE

3,695,919

METAL COATING PROCESS

Filed Nov. 20, 1970



FIG. 1.



FIG. 2.

INVENTOR.  
KENNETH J. BRONDYKE  
By  
*Arnold B. Silverman*  
Attorney

1

3,695,919

**METAL COATING PROCESS**

Kenneth J. Brondyke, Oakmont, Pa., assignor to  
Aluminum Company of America, Pittsburgh, Pa.  
Filed Nov. 20, 1970, Ser. No. 91,387

Int. Cl. B44d 1/34; C23c 1/00

U.S. CL. 117—52

9 Claims

**ABSTRACT OF THE DISCLOSURE**

A process for aluminizing an article by immersion in a vessel containing a bath of molten aluminum. Providing at least one foraminous refractory brick impregnated with a flux material having a density less than the molten aluminum bath. Introducing the brick into the vessel in contact with the aluminum to initiate discharge of the flux from the refractory brick into the aluminum. Retaining the brick in the vessel for a sufficiently long period of time to establish a thin film of the flux on the surface of the molten aluminum. Subsequently introducing the article to be aluminized into the molten aluminum and retaining it therein for a period of time sufficient to coat the article with the molten aluminum. Thereafter removing the article at a sufficiently low rate of speed to cause flux pickup to provide a flux coating on the coated article and thereby minimizing oxide formation on the cooled part. The foraminous refractory brick is preferably thermally stable at the molten aluminum bath temperature and the flux preferably has a melting temperature not less than the temperature of the molten aluminum bath.

**BACKGROUND OF THE INVENTION****Field of the invention**

This invention relates to the aluminizing of articles and more specifically a process for improving the uniformity of the aluminum coating on the article by means of a carefully applied flux film which is established on the surface of the molten aluminum.

**Description of the prior art**

The advantageous use of aluminizing to coat numerous products made of ferrous materials, titanium or other metals has long been known. Such coatings not only provide an attractive exterior appearance, but also provide resistance to corrosion, acid attack and oxidation. In addition, increased reflectivity and electrical conductivity may be provided. Numerous means of applying such an aluminum coating to an article have been known. Included within the known systems are spraying, cladding, electroplating, casting and immersion of the article in a molten aluminum bath.

One of the principal problems encountered in aluminizing systems is the need to improve the uniformity of coating thickness. This problem is particularly acute with respect to irregularly configurated articles.

In general, the known systems of immersion or hot dip aluminizing have followed the same general pattern. After some sort of preliminary cleaning which may be effected mechanically or in an alkaline solution the article is subsequently pickled. The article is then fluxed, dried and immersed in molten aluminum. After a sufficient period of immersion to accomplish the desired coating thickness while preventing excess formation of the aluminum-ferrous intermetallic compound or other intermetallic compounds the article is then removed. It is then conventional to attempt to remove excess aluminum adhering to the article either manually or mechanically as by draining, spinning, vibrating or centrifuging.

2

One of the principal contributing causes of the lack of uniformity of aluminum coating on an aluminized article is the difficulty in obtaining optimum wetting of the article while it is immersed in the molten aluminum bath and effecting substantially complete removal of any excess material by a subsequent operation. This problem provides both technical and economical obstacles to broader commercial use of hot dip aluminizing.

**SUMMARY OF THE INVENTION**

The process of this invention has solved the above enumerated problems with respect to uniformity of aluminum coating in hot dip aluminizing. In general, this invention contemplates providing a foraminous refractory brick which is mechanically stable under the thermal and metallurgical conditions encountered in the aluminum bath. A flux material which has a density less than the molten aluminum bath is then impregnated into the foraminous refractory brick. The brick, which may have a density greater than, less than or substantially equal to the molten aluminum bath, is then introduced into the vessel of molten aluminum. The brick is retained in the vessel for at least a sufficiently long period of time to establish a thin film of the flux on the surface of the molten aluminum. Subsequently an article to be aluminized is immersed in the molten aluminum bath and retained therein for a sufficiently long period of time to coat the article with molten aluminum. The article is removed at a sufficiently slow rate of speed as to cause flux pickup and provide a flux coating on the coated article. This flux coating minimizes oxide formation on the cooled part, contributes to improve flow characteristics of the aluminum and permits increased ability to remove excess aluminum.

The flux material preferably has a melting temperature approximately the temperature of the molten aluminum and provides a substantially continuous flux film on the surface of the bath. This film preferably has a thickness of less than about  $\frac{1}{32}$  inch.

After removal of the excess aluminum, the article with a solidified aluminum coating may then be cleansed to remove residual flux therefrom.

It is an object of this invention to provide a process of aluminizing an article which will permit ready removal of excess aluminum as a result of a unique fluxing operation.

It is a further object of this invention to provide a foraminous refractory brick which has been impregnated with a flux material adapted to be released when the brick is immersed in the molten aluminum bath to establish a thin flux film for coating an article being removed from the molten aluminum bath.

It is a further object of this invention to provide a method of controlling the rate of release of a flux material to provide a thin film thereof on the surface of the molten aluminum bath.

It is yet another object of this invention to provide such a process which is adapted for use with conventional aluminizing equipment and materials and may be economically introduced into such a system.

These and other objects of the invention will be more fully understood from the following description of the invention on reference to the illustrations appended hereto.

**65 BRIEF DESCRIPTION OF THE DRAWINGS**

FIG. 1 is a partially schematic sectional elevation of a vessel containing molten aluminum and a refractory brick of this invention.

FIG. 2 is a flow chart illustrating one means of practicing the process of this invention.

## DESCRIPTION OF THE PREFERRED EMBODIMENTS

As used herein, the term "aluminum" shall refer to aluminum of any grade and aluminum base alloys wherein aluminum consists of not less than 80% by weight of the total composition.

The process of this invention contemplates the hot dip aluminizing of articles made of ferrous materials, titanium, refractory metals and other suitable materials. As will be described in greater detail below, the invention provides a thin film of flux material on the surface of an aluminum bath by a unique controllable method which involves impregnating of a foraminous brick element with a flux material. The brick is adapted to retain its unitary structure and release the flux material at a predetermined rate when the brick is placed in or on the molten aluminum bath. The impregnated brick may be provided with a density greater than the density of the molten aluminum bath and sinks to the bottom of the bath as shown in FIG. 1 to discharge the material therefrom. Alternatively, the brick in impregnated form may have a density less than that of the molten aluminum bath and may float thereon and discharge flux from said position. Finally, a density equal to that of the bath may also be provided.

Referring now to FIG. 1, it is seen that a vessel 2 has a lining 4 which may be of refractory or other suitable material, an outer steel material 8 and an interposed insulating material 6. The vessel 2 contains a charge of molten aluminum 10. Submerged within the vessel is a foraminous brick 12 from which is being discharged flux 14 which migrates upwardly to form flux film 16 on the surface of the molten aluminum 10. (A brick 12a having a density less than that of the molten aluminum is illustrated in dotted form in FIG. 1.)

In fabricating the brick 12, it is preferred that it be made from a refractory material which is foraminous in nature and has a bulk density range from about 30 lbs./ft.<sup>3</sup> to 145 lbs./ft.<sup>3</sup>. The brick must have such thermal and mechanical properties as to resist excessive fragmentation or other forms of destruction of its integrity. The size of brick selected and the number inserted within any vessel will depend in part upon the porosity or permeability of the material, the area of the aluminum surface upon which the film will be established, the film thickness desired and the relationship between the temperature of the molten aluminum and the melting point of the flux material. The porosity of the brick will generally range from about 20 to 85%.

In selecting an appropriate flux material for use in this process in general it is desirable to select a material which will have a melting point approximating that of the temperature of the molten aluminum bath and preferably equal to or greater than the bath temperature. A flux melting temperature from about 10 degrees Fahrenheit below the temperature of the molten aluminum bath to about 15 degrees Fahrenheit above the bath temperature may be used. It is preferred to select a material having a melting point of about five degrees Fahrenheit below the bath temperature to about five degrees above the bath temperature. The molten aluminum bath depending upon alloy and weight characteristics sought and the material of the article to be coated will frequently be operated at a temperature of about 1275 to 1400° F. If an increase in the rate of discharge of flux from the refractory brick is desired, a melting point about 5 to 25° F. above the temperature of the molten aluminum bath is preferred. Numerous types of fluxes may be employed in the practice of this invention. One suitable form of flux is of the type employing sodium chloride, potassium chloride and potassium aluminum fluoride. Other suitable compositions are shown in U.S. Pats. 2,569,097, 2,544,670 and 2,544,671.

In order to establish the desired flux film position the flux must have a density less than that of the molten

aluminum bath. It is desired to provide a very thin film of the flux material on the surface of the bath. This film may be thought of as being preferably less than  $\frac{1}{32}$  inch in thickness and adapted to coat an emerging aluminum coated article in order to provide for efficient mechanical removal of excess aluminum and thereby establish a coating of uniform thickness.

As is shown in the flow diagram of FIG. 2, one convenient means of impregnating the brick with the flux is to provide for immersion of the brick in a molten flux bath and retention therein for the period necessary to accomplish the absorption. This has frequently been found to require one-half hour or more. The brick may then be removed. Before immersion in the molten aluminum bath, the impregnated brick is preferably subjected to heat in order to drive off any sorbed moisture.

## Example

20 A flux formulation consisting of 62.7% sodium chloride, 32.3% potassium chloride and 5% potassium aluminum fluoride was provided in a vessel and maintained at a temperature of 1400° F. A number of refractory bricks were immersed in the molten salt mixture and held therein for a one hour period. The bricks were removed and heated to drive off any sorbed moisture. They were found to have increased in weight by approximately one pound.

Referring once again to FIG. 2 and the flow diagram 30 shown therein, the article to be aluminized will first be subjected to a conventional cleaning operation which may include mechanical cleaning, alkaline cleaning and pickling. The article is then coated with an aluminizing flux material as by immersion in an aqueous solution and is subsequently dried. After the refractory brick has been in the molten aluminum bath for a sufficient period of time to provide the desired flux film on the bath surface, the article is immersed in the bath sufficiently far as to be entirely beneath the aluminum surface. The article is retained in the bath for a sufficient period of time to provide the optimum desired coating thickness and coating characteristics in terms of control over the quantity of intermetallic compounds formed between the aluminum coating material and the metal material of which the article is composed. The article is then withdrawn from the 40 bath at a sufficiently slow rate of speed to permit flux pick-up and provide a flux coating on the article. The presence of the flux coating on the article provides a means of reducing harmful oxidation on the aluminum surface of the emerging article and reduces influence of the oxide film or surface tension of the aluminum to provide for greater flowability and more efficient mechanical removal of the excess aluminum. This results in a more uniform coating thickness and appearance.

50 After removal from the molten aluminum bath, the article is subjected to a manual or mechanical process stage which serves to remove excess aluminum. This may be accomplished by draining, spinning, centrifuging or other desired means. It is the thin, preferably substantially continuous, film of flux material which serves to protectively surround the aluminum coating and establishes the desired free flow of the aluminum to provide discharge of the excess material. In addition, the presence of an oxide inhibiting flux also serves to prevent undesired discoloration which tends to impair the desired uniform surface appearance of the article.

55 The aluminum coating on the article may then be permitted to solidify. After solidification has occurred, the article may be cleaned to remove the residual flux present on the surface. This is preferably accomplished by means of an aqueous solution which may be a quench in water having a temperature of about 50° F. to 180° F. The higher temperatures within this range are preferred as increased solubility of the flux in the aqueous solution results.

It will therefore be appreciated that the process of this invention provides a means of effectively controlling the surface tension of the aluminum on the emerging coated product and restricting oxidation thereof. This contributes to ready removal of excess material in order to provide uniform coating thickness and aesthetically pleasing surface characteristics. All of this is accomplished by impregnating a refractory brick with a suitable flux material which is adapted to migrate to the surface of the molten aluminum bath and establish a thin film thereon. 10 The process may be employed with conventional hot dip aluminizing equipment and is readily adaptable to use with various size molten metal bath vessels as bricks in various sizes and numbers may be employed therein.

It will also be appreciated that the impregnated bricks 15 may be prepared in advance of the aluminizing operation and provide a means of accurately controlling the amount of flux charged into a vessel and thereby controlling the film thickness and amount of flux dissipation as the process is performed on a larger number of articles.

Whereas particular embodiments of the invention have been described above for purposes of illustration, it will be evident to those skilled in the art that numerous variations of the details may be made without departing from the invention as defined in the appended claims.

Having thus described my invention and certain embodiments thereof, I claim:

1. A process of aluminizing a metal article, comprising providing a vessel containing a molten aluminum bath, providing at least one foraminous refractory brick impregnated with a flux material, 30 introducing said brick into said vessel in contact with said aluminum to initiate discharge of said impregnated flux from said refractory brick into said aluminum without appreciable physical destruction of said foraminous refractory brick, 35 retaining said brick in said vessel for a sufficiently long period of time to establish a substantially continuous thin film of said flux on the surface of said molten aluminum while avoiding appreciable physical destruction of said foraminous refractory brick, 40 subsequently introducing said metal article to be aluminized into said molten aluminum and retaining it therein for a sufficient period of time to coat said article with said molten aluminum, and 45 thereafter removing said article at a sufficiently slow rate of speed as to cause flux pickup to provide a flux coating on said coated article.
2. The aluminizing process of claim 1 wherein said refractory brick has a lower density than said 50 molten aluminum, and said brick is floating on the surface of said molten aluminum bath during discharge of flux therefrom.
3. The aluminizing process of claim 1 including

providing said impregnated foraminous refractory brick by immersing said foraminous brick in a molten flux bath for a sufficient period of time to effect impregnation of a predetermined quantity of said flux and subsequently heating said brick to drive off any sorbed moisture.

4. The aluminizing process of claim 1 wherein said refractory brick has a porosity of about 20 to 85%, said flux has a melting temperature of about 10 degrees Fahrenheit below the temperature of said molten aluminum to about 15 degrees Fahrenheit above the temperature of said molten aluminum, and said refractory brick is physically stable and remains unitary at the temperature of said molten aluminum.
5. The aluminizing process of claim 4 wherein said refractory brick has a higher density than said molten aluminum bath, and said brick is positioned below the surface of said molten aluminum bath during discharge of flux therefrom.
6. The aluminizing process of claim 1 wherein said flux has a melting temperature of about 5 to 25° F. above the temperature of said molten aluminum bath and said refractory brick has a density of about 30 lbs./ft.<sup>3</sup> to 145 lbs./ft.<sup>3</sup>.
7. The aluminizing process of claim 6 wherein after withdrawal of said coated article from said molten aluminum bath but prior to full solidification of said aluminum coating, mechanically removing the excess of said aluminum coating to establish a substantially uniform coating on said article.
8. The aluminizing process of claim 7 wherein said film of said flux has a thickness of not greater than  $\frac{1}{32}$  of an inch, and subsequent to full solidification of said aluminum coating cleansing said coated article by means of an aqueous solution to remove residual flux therefrom.
9. The aluminizing process of claim 8 wherein said residual flux removal is accomplished by immersing the coated article in water having a temperature of about 50° F. to 180° F.

#### References Cited

#### UNITED STATES PATENTS

|           |         |        |         |
|-----------|---------|--------|---------|
| 3,037,880 | 6/1962  | Hanink | 117—52  |
| 3,486,884 | 12/1969 | Baille | 75—68 R |

ALFRED L. LEAVITT, Primary Examiner

J. A. BELL, Assistant Examiner

#### U.S. CL. X.R.

117—114 C, 131; 75—68, 93 AC, 94; 148—26